

Sept. 7, 1943.

J. E. KIRBY ET AL

2,328,652

PROCESS OF COLOR PHOTOGRAPHY AND COMPOSITIONS THEREOF

Filed April 18, 1941



INVENTORS.

James E. Kirby  
David M. McQueen

BY

Lynn B. Morris  
ATTORNEY

## UNITED STATES PATENT OFFICE

2,328,652

PROCESS OF COLOR PHOTOGRAPHY AND  
COMPOSITION THEREOF

James Emory Kirby and David M. McQueen,  
Wilmington, Del., assignors by mesne assignments, to E. I. du Pont de Nemours & Company,  
Wilmington, Del., a corporation of Delaware

Application April 18, 1941, Serial No. 339,244

21 Claims.

(Cl. 95—6)

This invention relates to color photography. More particularly it relates to photographic color processes utilizing N-homophthalylamines and to compositions therefor. Still more particularly it relates to dye image formation in photographic elements by color-coupling development in the presence of N-homophthalylamines and to compositions containing such N-homophthalylamines. The invention also relates to novel N-homophthalylamines and to their preparation and incorporation in photographic compositions.

This invention has for an object the production of new photographic compositions and elements which can be used in the formation of dye images in processes of color photography. A further object is to provide colloid emulsion layers which contain N-homophthalylamines. A further object is to provide new N-homophthalylamines which form dye images of improved tintorial strength and color upon color coupling development of silver halide images. A still further object is to provide new N-homophthalylamines which are non-migratory in colloid layers. Another object is to provide new photographic developer solutions containing novel N-homophthalylamines. Still another object is to provide new chemical compounds, a new use for homophthalic anhydride, new dye intermediates and a general advance in the chemical and related arts.

It has been found that the N-homophthalylamines, especially N-homophthalyl aromatic amines produce dye images of excellent density by color coupling in photographic color processes. To be more specific, it has been found the N-homophthalylamines can be used in processes of producing photographic color pictures with the aid of color coupling development of silver salt images wherein these dye intermediates are present in the developer solutions or in colloid layers of color yielding photographic elements, and that images of excellent dye purity are formed.

The N-homophthalylamines when used in accordance with one aspect of this invention can be dissolved in a suitable solvent, e. g. a water-soluble solvent such as methanol, ethanol and acetone or a dilute aqueous alkali solution which may contain small amounts of said organic solvents and added to a developer solution containing a color coupling developing agent, such as an aromatic primary amino developing agent or a hydrazine. A photographic element containing

a reducible or developable silver salt image is immersed in the solution and development allowed to proceed until the desired amount of color is deposited. The film is removed, washed and finally the silver and any undeveloped silver salts are removed. The resulting film contains a dye image in a color the hue of which depends upon the particular N-homophthalylamine and developing agent chosen.

In a further aspect of the invention, immobile N-homophthalylamines are incorporated in organic colloid dispersions which are then deposited upon a support, e. g. a film base to form a thin layer to carry an image. A practical manner involves dispersing the N-homophthalylamines in an aqueous alkali, usually with the addition of a small amount of a water-soluble organic solvent, and admixing it with the organic colloid which may be a photographic emulsion containing a reducible silver salt. The dispersions may then be cast or deposited on a suitably subbed film base or an organic colloid layer, a similar layer, or a water-permeable membrane to form, for example, single or multilayer elements for photographic color processes.

Silver halide emulsions containing one or more of the above color formers or dye intermediates may be worked up in the usual manner. One or more emulsion layers being superposed on one or both sides of transparent supports as desired. The layers may be used for color photography and for such purposes the layers are sensitized respectively for different regions of the spectrum. They may also be used in conjunction with the usual cyanine, carbocyanine, pseudocyanine, cyanine, carbocyanine, merocyanine, etc. dyes which are used to extend the sensitivity of silver halide emulsions.

The development process used in carrying out this invention may be applied either to latent images in an emulsion layer composed of silver halides which have been exposed and which may or may not contain the novel color formers hereof. Or, it may be applied to the residual unaltered silver salt left where an initial reduced silver image has been rendered incapable of influencing color coupling or dissolved away as in a reversal process of development. Or it may be applied to a reducible silver salt image which remains after the removal of unaltered silver halides by means of solvents and subsequent conversion of the developed silver image to a silver

salt by means of known silver bleaching agents.

An important group of useful N-homophthalylamines have the following general formula:

(1)



wherein R is a hydrocarbon radical which may be aliphatic, cycloaliphatic or aromatic, this R may be a primary, secondary, tertiary, iso, or branched chain alkyl, having preferably 8 to 18 carbon atoms; alkenyl preferably 8 to 18 carbon atoms, cycloaliphatic, aralkyl such as benzyl, chlorobenzyl and menaphthyl, and aryl, e. g. phenyl, chlorophenyl, naphthyl, dodecylphenyl. The hydrocarbon radicals attached to the nitrogen atom may be substituted or unsubstituted and contain neutral or salt-forming substituents such as hydrocarbon radicals, halogen atoms, e. g. chlorine, bromine, NH<sub>2</sub>, NHR, NRR', OH, OR, SO<sub>3</sub>H, COOH (wherein the Rs constitute hydrocarbon radicals of the same type as R in Formula 1).

The compounds of Formula 1 can be made by reacting at least one mol of homophthalic anhydride with about one mol of a primary amine and recovering the N-homophthalylamine. The reaction is preferably carried out by heating the reactants at a temperature of 100° to 250° C. for a short period followed by isolating the compound by precipitation, extraction, distillation, etc. steps, and purifying it by recrystallization, etc. When the primary amine is not a liquid at moderate temperatures, it is desirable to add an inert organic diluent or solvent. Suitable solvents include hydrocarbons, e. g. benzene, toluene, xylenes, hexane, etc., chlorinated hydrocarbons, e. g. carbon tetrachloride, trichloroethylene, tetrachloroethane, chlorobenzene, etc., ethers, e. g. dioxane, etc.

The invention as is apparent from the above disclosure is not limited to the use of any particular type of primary amine for the preparation of the N-homophthalylamines. On the contrary, any mono- or poly-amine containing one or more unsubstituted amino groups can be reacted in similar manner. Aliphatic, cycloaliphatic, or alicyclic, aromatic and heterocyclic mono-, di- and poly-amines can be used. In the case of the di- and poly-amines, in general about one mol of homophthalic anhydride should be used for each primary amino group. When primary diamino-alkanes or arylenediamines are used, bis-homophthalylamines are formed which are believed to constitute a new class of compounds.

The invention will be further illustrated but is not intended to be limited by the following examples, wherein the parts stated are parts by weight:

#### Example I

Four parts of aniline and 4 parts of homophthalic anhydride of formula



are mixed in a reaction vessel and heated slightly. The temperature is gradually raised during one

hour to 150° and the water formed in the reaction driven off. After cooling, the solid cake of reaction product is ground up and washed thoroughly with ether. After crystallization from ethanol, a white solid melting at 188-190° C. is obtained. The amount of nitrogen found by analysis is 5.71% while that calculated for N-homophthalylaniline was 5.90%. The probable formula is

10



15

The product is soluble in alcohol, acetone, and dilute aqueous alkaline solutions. A color developer is prepared by dissolving 2 parts of sodium carbonate, 0.1 part sodium sulfite, and 0.2 part p-aminodiethylaniline hydrochloride in 100 parts water. To this is added 0.25 part of N-homophthalylaniline dissolved in 10 parts acetone. A film element bearing an image in silver ferrocyanide in a gelatin layer is immersed in the resulting mixture for 8 to 10 minutes, after which it is washed in running water, bleached in 4% potassium ferricyanide solution and fixed in 25% sodium thiosulfate solution. This treatment removes all silver and silver salts and leaves a clear, bright blue dye image in said layer.

#### Example II

A film element bearing a silver ferrocyanide image in a gelatin layer is treated for 5 to 8 minutes with a color developer, prepared by dissolving 4.5 parts p-aminophenol, 20 parts sodium carbonate, and 1 part sodium sulfite in 1000 parts water, to which is added a solution of 0.2 part N-homophthalylaniline in 10 parts ethanol. After removal of silver and silver salts from the film, a reddish-purple image remains in said layer.

#### Example III

Five parts of homophthalic anhydride and 5 parts of 2,5-dichloroaniline are mixed and heated in an open glass vessel on a metal bath. The temperature is slowly raised until the material becomes liquid after which it is maintained at 140-150° C. until the mixture solidifies (approximately 3 hours). During this heating water is given off. The reaction mass is crystallized from ethyl acetate and a white solid melting at 165-167° C. is obtained. This compound contains 22.45% chlorine by analysis, whereas that calculated on the basis of the following formula, N-homophthalyl-2,5-dichloroaniline is 23.20%.

60



65

Two tenths part of the solid is dissolved in 5 parts 1% sodium carbonate solution containing 1 part methanol and the solution added to 50 parts of an alkaline p-aminodiethylaniline developer solution. The resulting solution is used to develop a silver bromide image in a gelatin layer of a photographic element. After removing silver and silver salts, a brilliant blue image is obtained.

#### Example IV

Three and five-tenths parts beta-naphthyl-

amine and 4 parts homophthalic anhydride are melted together in an open glass vessel and then heated for one-half hour at a temperature of 180-200° C. At the end of this time the mixture solidifies. Crystallization from ethyl acetate yields a white solid of melting point 212-4° C. Incorporation of this compound, N-homophthalyl- $\beta$ -naphthylamine, having the formula:



in an aqueous alkaline color developer solution prepared with 4 - amino-3-methyl-N-diethyl-aniline as the active developer constituent yields a blue image in an element when treated after the manner set forth in Example I.

*Example V*

Four parts homophthalic anhydride and 6 parts of dodecylamine are mixed at room temperature. The reaction is slightly exothermic. The mixture is then heated at 150-200° C. for one hour, and the resulting solid is crystallized from an ether-petroleum ether mixture and finally recrystallized from methanol. The product melts at 93-95° C. with preliminary softening at 60° C. and contains 4.04% nitrogen. The nitrogen content calculated for N-homophthalyldodecylamine is 4.25%. This compound is dissolved in a mixture of dilute sodium carbonate solution and methanol and incorporated in a gelatino silver chloride-bromide photographic emulsion. After coating on a cellulose nitrate film base, the resulting film is exposed and developed with p-aminodiethylaniline developer. A blue dye image is formed in situ with the metallic silver image.

*Example VI*

The reaction mixture obtained by heating together 1.8 parts of homophthalic anhydride and 1.3 parts of octylamine for two hours at 150° C. is dissolved in 20 parts ethanol and incorporated in 250 parts of a panchromatic photographic gelatino-silver halide emulsion. The resulting emulsion is coated on a cellulose acetate film base and the film exposed and developed with an aqueous alkaline p-phenylenediamine developer. A blue colored image results.

In place of the specific compounds set forth in the preceding examples may be substituted a large number of other N-homophthalylamines having the above-described structure and constitution in similar amounts. The compounds which are of utility in producing photographic dye images fall in general into two classes: (1) Compounds of low molecular weight which penetrate gelatin films freely. These are most suitable for incorporation in solutions of known color developers, and (2) high molecular weight compounds which are immobile in gelatin layers and which are exemplified by N-homophthalyl-dodecylamine. These are most suitably incorporated in the photographic emulsion itself. Besides immobilization of these compounds by attachment of a long chain aliphatic group which has been exemplified, the compounds may be made non-removable from photographic gelatino-silver halide layers by attaching a polymeric group, or a high molecular weight aromatic

group. Of these immobile types, we prefer the N-homophthalylamines substituted on the nitrogen atom with a long chain alkyl group containing at least 8 carbon atoms such as N-homophthalyloctadecylamine and N-homophthalyl-para-dodecylaniline.

Additional suitable N-homophthalylamines of the above-described types which can be prepared from homophthalic anhydride and the corresponding primary amines as herein disclosed, include the following compounds:

1. N-homophthalyl-alpha-naphthylamine
2. N-homophthalyl-p-aminomethylaniline
3. N-homophthalyl-p-anisidine
4. N-homophthalyl-p-aminophenol
5. N-homophthalyl-p-toluidine
6. N-homophthalyl-m-aminobenzoic acid
7. N-homophthalylmetanilic acid
8. N-homophthalyl-m-nitro-p-toluidine
9. N-homophthalyl-p-nitroaniline
10. N-homophthalyl-o-chloroaniline
11. N-homophthalyl-p-aminobiphenyl
12. N-homophthalylbenzylamine
13. N-homophthalylfurfurylamine
14. N-homophthalyl-2-ethylhexylamine
15. N-homophthalylisobutylamine
16. N-homophthalylethylamine
17. N-homophthalyl-n-octadecylamine
18. N-homophthalyl-n-hexadecylamine
19. N-homophthalyl-12-aminostearamide
20. N-homophthalyl-epsilon-aminocaproic acid
21. N-homophthalylcyclohexylamine
22. N,N'-bis-homophthalylethylenediamine
23. N,N' - bis - homophthalylhexamethylenediamine
24. N,N' - bis - homophthalyldecamethylenediamine
25. N,N' - bis-homophthalyltriglycoldiamine
26. N,N' - bis-homophthalyl-m-phenylenediamine
27. N,N' - bis-homophthalyl-p-phenylenediamine
28. N,N' - bis - homophthalyl - m - phenylenediaminesulfonic acid
29. N,N' - bis - homophthalyl - p - phenylenediaminesulfonic acid
30. N,N' - bis-homophthalylbenzidine
31. N,N' - bis-homophthalyldianisidine
32. N,N' - bis-homophthalyltoluidine

It is characteristic of the products that they are all soluble to a greater or lesser extent in dilute aqueous alkaline solutions and from such solutions they may be readily incorporated into the weakly alkaline photographic emulsion where they manifest high compatibility. This solubility in alkali also is of advantage in that they may be incorporated into weakly alkaline photographic developer solutions. Although in general it is not necessary, the compounds may also be dissolved in water-miscible organic solvents

such as acetone or alcohol and added to the photographic emulsion or developer as desired.

A comparison between homophthalimide and the N-homophthalylamines of the present invention is shown in the accompanying drawing wherein curve A represents the density of the dye obtained by developing a photographic film element containing a developable silver salt image in a gelatin emulsion layer with p-aminodiethylaniline developer containing homophthalimide, and curve B represents the density of the dye obtained by developing a similar photographic film element with the same developer containing N-homophthalylaniline. The great difference in saturation and purity is an unexpected result, and the incomparably superior properties of the

compounds of the present invention suggest that there is an actual difference in structure between them and homophthalimide. This is entirely probable since it is well known that homophthalimide has the possibility of existing in the form of the isoquinoline derivative.



while the homophthalylamines cannot so exist because of the substituent groups on the nitrogen atom.

While all the homophthalylamines are of utility in the preparation of color photographic elements, we prefer the homophthalyl aromatic amines because they yield dyes having higher saturation, greater brilliancy, and purity. Another class of preferred compounds consists of the N,N'-bis-homophthalylamines which are readily prepared by reaction of two molecules of homophthalic acid or homophthalic anhydride with one molecule of a primary diamine. The presence of the two coupling residues in the one molecule of color former with these compounds is believed to confer enhanced color intensity and brilliancy. In many cases the high molecular weight of the bis-homophthalylamines results in a resistance to diffusion in gelatin layers. A similar resistance to diffusion is encountered in the homophthalyl polymeric amines such as poly(p-aminostyrene) and its interpolymers, for example, such as are described in British Patent 524,996.

The dye intermediates are useful in various types of color processes wherein dye images are produced by color-forming development and azo coupling processes and processes including both color-forming development and azo coupling of the same color formers. They may be used in conjunction with various types of reducible silver salt images, including silver halides, such as the chloride, bromide, chlorobromide, chloro-bromo-iodide, etc. images; bleached silver images, i. e. silver ferrocyanide, silver-copper-chloride, silver-chromium-chloride, as well as silver chromate and other water insoluble silver salts. The images formed by the exposure of bichromated gelatine are also reduced by the color-forming developers described above, yielding blue dye images.

The compounds of the present invention are of considerable utility in the preparation of azo dyes. The homophthalylamines are energetic couplers and couple even with weakly coupling diazonium salts such as benzenediazonium chloride. The shade of the dyes obtained varies considerably with the diazonium salts chosen, but in general lies between yellow-orange and bluish-red.

In place of the specific developing agents described in the above examples can be substituted a large number of other color-developing agents containing an unsubstituted amino group. Suitable additional agents are described in U. S. Patents 2,182,815, 2,189,817, 2,191,037 and 2,200,924.

The silver salt images can also be developed with hydrazine developers in like manner to produce azo dye images. Suitable developers are described in U. S. Patent 2,220,929.

In addition, a silver halide emulsion layer containing one of the herein described N-homophthalylamines which has been exposed and developed to a silver image and fixed can be treated

with a diazo or tetrazo, etc. salt and converted into a colored image by the process of U. S. Patent 1,517,049.

The compounds hereof can also be used in photographic color processes involving azo coupling. They couple readily in emulsion layers with diazotized aromatic amines and give azo dye images of good color and strength. The new compounds give azo dyes which are of utility in the arts.

The substitution of a hydrocarbon residue on the nitrogen atom of homophthalimide has been shown to result in greatly improved color obtained upon color development of a silver salt in the presence of such compounds. The dyes thus obtained show greatly improved brilliancy and saturation over the unsubstituted homophthalimide itself as is shown by the curves in the accompanying drawing.

Various types of organic colloids can be used as the binding agents for the dispersions or emulsions and colloid layers described herein. Suitable colloids exhibiting high viscosity characteristics and appreciable jelly strength which are compatible with the N-homophthalylamines and can be used as binding agents in place of gelatin include albumin, agar-agar, Irish moss, synthetic resins, e. g. polyvinyl alcohol, etc.

As many apparently widely different embodiments of this invention may be made without departing from the spirit and scope thereof it is to be understood that the invention is not to be limited except as defined by the appended claims.

We claim:

1. A photographic element bearing at least one water-permeable colloid layer having dispersed therethrough an N-homophthalylamine.
2. A photographic element bearing at least one water-permeable colloid layer having dispersed therethrough an N-homophthalylamine which contains in its molecule a radical which imparts thereto fastness to diffusion with respect to said colloid layer while retaining solubility in aqueous liquids.
3. A photographic element bearing at least one water-permeable colloid layer having dispersed therethrough an N-homophthalylaromaticamine.
4. A photographic element bearing at least one water-permeable colloid layer having dispersed therethrough an N-homophthalylarylamine.
5. A photographic element bearing at least one water-permeable colloid layer having dispersed therethrough an N-homophthalalkylamine having at least 8 carbon atoms in the aliphatic chain.
6. A photographic element bearing at least one water-permeable colloid layer having dispersed therethrough an N,N'-bis-homophthalylamine.
7. A photographic element bearing at least one water-permeable colloid layer having dispersed therethrough an N-homophthalylamine and a reducible silver salt.
8. An element as set forth in claim 7 wherein said amine contains in its molecule a radical which imparts thereto fastness to diffusion with respect to said colloid layer while retaining solubility in aqueous liquids.
9. A photographic developer comprising an aqueous solution containing a color coupling developing agent and an N-homophthalylamine.
10. A photographic developer comprising an

aqueous alkaline solution containing an aromatic primary amino developing agent and an N-homophthalylamine.

11. A photographic developer comprising an aqueous alkaline solution containing an aromatic primary amino developing agent and an N-homophthalylarylamine.

12. The process which comprises developing a photographic element containing a reducible silver salt image record with a color coupling developing agent in the presence of an N-homophthalylamine.

13. A process as set forth in claim 12 wherein said amine nucleus contains a solubilizing group.

14. The process which comprises developing a photographic element containing a reducible silver salt image record with a color coupling developing agent containing a primary amino group in the presence of an N-homophthalylarylamine.

15. The process which comprises developing a photographic element containing a reducible silver salt image record with a color coupling developing agent containing a primary amino group in the presence of an N-homophthalylkylamine wherein the aliphatic hydrocarbon radical contains at least 8 carbon atoms.

16. The process which comprises developing a

photographic element containing a reducible silver salt image record with a color coupling primary aromatic amino developing agent in the presence of N-homophthalylaniline.

17. A photographic developer comprising an aqueous alkaline solution containing an aromatic primary amino developing agent and N-homophthalylaniline.

18. The process which comprises developing 10 a photographic element containing a reducible silver salt image record with a color coupling primary aromatic amino developing agent in the presence of N-homophthalyl-m-amino benzoic acid.

19. A photographic developer comprising an aqueous alkaline solution containing an aromatic primary developing agent and N-homophthalyl-m-amino benzoic acid.

20. The process which comprises developing a photographic element containing a reducible silver salt image record with a color coupling primary aromatic amino developing agent in the presence of N-homophthalyldodecylamine.

21. A photographic element bearing at least 25 one water permeable colloid layer having dispersed therethrough N-homophthalyldodecylamine.

JAMES EMORY KIRBY.  
DAVID M. MCQUEEN.